

## UNITED STATES PATENT OFFICE

2,150,704

## PHOTOGRAPHIC REVERSAL PROCESS

Joseph C. Ville, Rochester, N. Y., assignor to Eastman Kodak Company, Rochester, N. Y., a corporation of New Jersey

No Drawing. Application September 3, 1937,  
Serial No. 162,331

10 Claims. (Cl. 95—88)

This invention relates to a photographic reversal process and particularly to agents which fog the unexposed portions of a sensitive photographic layer prior to reversal.

5 In making positive photographic images by reversal from negative photographic images, it is customary to bleach or remove the metallic silver image before fixing the photographic element and while sensitive silver halide remains in the element, and then to re-expose the sensitive layer and develop a positive image in the originally unexposed portions of the element. Methods have been proposed for fogging the sensitive layer after the first development so that the second 10 exposure is unnecessary and then developing a positive image in the usual way. Many of the methods previously suggested for this purpose were undesirable for various reasons, among which were that some of the fogging agents required the use of special developers for formation of the positive image with an attendant limitation on the physical properties of the final positive image, while others tended to produce a stain in the film or paper in which the image was formed.

15 It is accordingly an object of the present invention to provide a reversal process in which positive images may be produced on development without a second exposure. A further object is to provide a reversal process in which an ordinary developer may be used in the second development. Other objects will appear from the description of my invention.

20 These objects are accomplished in the present invention by using as the fogging agents or nucleus-forming agents prior to the second development, substituted hydrazine derivatives, especially the aromatic-ring-substituted derivatives. Specific compounds which I have found suitable are semicarbazide, phenyl hydrazine, acetyl phenyl hydrazine, hydrazino benzoic acid and naphthyl hydrazine. The hydrazine may, therefore, be substituted with various groups, such as an aromatic ring of either the benzene, or the naphthalene series, or a carbamyl group, and these groups may themselves contain substituent groups. The carbamyl group is 25  $\text{NH}_2\text{CO}-$ , so that hydrazine substituted with this group would have the structural formula  $\text{NH}_2\text{CO}-\text{NHNH}_2$  (semicarbazide).

30 The following is a specific example of one method of forming a reversed positive image according to my invention.

35 A sensitive photographic element which may be a plate, film, or paper is exposed to a subject

in the usual way and is then developed in a solution having the following composition:

|                             |       |      |
|-----------------------------|-------|------|
| Water                       | liter | .75  |
| Sodium sulphite, desiccated | grams | 48.8 |
| Hydroquinone                | do    | 24.4 |
| Boric acid                  | do    | 5.6  |
| Potassium bromide           | do    | 2.8  |
| Sodium hydroxide            | do    | 24.4 |
| Water                       | liter | 1    |

40 After development at 70° F. the film or paper is treated in the following solution at 65—70° F. for a sufficient length of time to bleach and remove the silver image formed by development without affecting the silver halide:

|                              |       |     |
|------------------------------|-------|-----|
| Water                        | liter | 1   |
| Potassium bichromate         | grams | 9.4 |
| Sulfuric acid (concentrated) | cc.   | 12  |

45 The film or paper is then washed and immersed in a clearing bath made up of 90 grams of sodium sulfite in 1 liter of water. The film or paper is then again washed and without being exposed to light is developed for 30 seconds in a developer having the same composition as for the first development, but having added thereto 10 grams of semicarbazide hydrochloride.

50 After development the film is again washed and dried although the fixing at this stage is not essential.

I have described my redeveloping solution as containing 10 grams of semicarbazide hydrochloride in 1 liter. However, the amount of hydrazine derivative used may be varied widely without departing from my invention.

55 Although I have described above the addition of my fogging or nucleating agent to the second developer, this compound may also be added to the clearing bath, if the clearing bath is made alkaline. In this case the fogging agent is used in the same concentration as in the developer, namely, that of about 10 grams per liter of solution.

It is to be understood that the above example is illustrative only and that my invention is to 45 be considered as limited only by the scope of the appended claims.

I claim:

1. The method of making a positive photographic image from a negative image in a photographic element without a second exposure to light, which comprises removing the negative image, treating the element in a bath containing as a nucleus-forming agent a hydrazine substituted with a group selected from aromatic ring 55

and carbamyl groups, and developing a positive image in the film.

5 2. The method of making a positive photographic image from a negative image in a photographic element without a second exposure to light, which comprises removing the negative image, treating the element in a bath containing a semi-carbazide as a nucleus-forming agent, and developing a positive image in the film.

10 3. The method of making a positive photographic image from a negative image in a photographic element without a second exposure to light, which comprises removing the negative image, treating the element in a bath containing a phenyl hydrazine as a nucleus-forming agent, and developing a positive image in the film.

15 4. The method of making a positive photographic image by reversal from a negative photographic image in a material having light-sensitive portions, which comprises bleaching the negative image in an aqueous solution of potassium bichromate and sulfuric acid, subjecting the sensitive element to the action of an aqueous solution of a hydrazine substituted with a group selected from aromatic ring and carbamyl groups as a nucleus-forming agent, and without exposing the element to light, developing a positive image in the film.

20 5. The method of making a positive photographic image by reversal from an element containing a visible negative image and a transparent, sensitive, positive image, which comprises removing the negative image, subjecting the element in the absence of an exposing light, to the action of an aqueous solution of a hydrazine substituted with a group selected from aromatic ring and carbamyl groups and developing a visible positive image in the element.

25 6. A photographic reversal process comprising forming a silver image in a gelatino-silver halide

emulsion layer, removing the silver image without affecting the remaining silver halide, subjecting the layer to the action of an aqueous solution of a hydrazine substituted with a group selected from aromatic ring and carbamyl groups as a nucleus-forming agent, and developing a positive image in the layer.

30 7. A photographic reversal process comprising forming a silver image in a gelatino-silver halide emulsion layer, removing the silver image without affecting the remaining silver halide, subjecting the layer to the action of an aqueous solution of semi carbazide as a nucleus-forming agent, and developing a positive image in the layer.

15 8. A photographic reversal process comprising forming a silver image in a gelatino-silver halide emulsion layer, removing the silver image without affecting the remaining silver halide, subjecting the layer to the action of an aqueous solution of a phenyl hydrazine as a nucleus-forming agent, and developing a positive image in the layer.

20 9. A photographic reversal process comprising forming a silver image in a gelatino-silver halide emulsion layer, removing the silver image without affecting the remaining silver halide, subjecting the layer to the action of an aqueous solution of hydrazino benzoic acid as a nucleus-forming agent, and developing a positive image in the layer.

25 10. A photographic reversal process comprising forming a silver image in a gelatino-silver halide emulsion layer, removing the silver image without affecting the remaining silver halide, subjecting the layer to the action of an aqueous solution of acetyl phenyl hydrazine as a nucleus-forming agent, and developing a positive image in the layer.

30 40 JOSEPH C. VILLE.

#### CERTIFICATE OF CORRECTION.

Patent No. 2,150,704.

March 14, 1939.

JOSEPH C. VILLE.

It is hereby certified that error appears in the printed specification of the above numbered patent requiring correction as follows: Page 2, second column, line 28, claim 9, strike out the syllable, words and syllable "tion of hydrazino benzoic acid as a nucleus-; and that the said Letters Patent should be read with this correction therein that the same may conform to the record of the case in the Patent Office.

Signed and sealed this 18th day of April, A. D. 1939.

Henry Van Arsdale

(Seal)

Acting Commissioner of Patents.

and carbamyl groups, and developing a positive image in the film.

5 2. The method of making a positive photographic image from a negative image in a photographic element without a second exposure to light, which comprises removing the negative image, treating the element in a bath containing a semi-carbazide as a nucleus-forming agent, and developing a positive image in the film.

10 3. The method of making a positive photographic image from a negative image in a photographic element without a second exposure to light, which comprises removing the negative image, treating the element in a bath containing a phenyl hydrazine as a nucleus-forming agent, and developing a positive image in the film.

15 4. The method of making a positive photographic image by reversal from a negative photographic image in a material having light-sensitive portions, which comprises bleaching the negative image in an aqueous solution of potassium bichromate and sulfuric acid, subjecting the sensitive element to the action of an aqueous solution of a hydrazine substituted with a group selected from aromatic ring and carbamyl groups as a nucleus-forming agent, and without exposing the element to light, developing a positive image in the film.

20 5. The method of making a positive photographic image by reversal from an element containing a visible negative image and a transparent, sensitive, positive image, which comprises removing the negative image, subjecting the element in the absence of an exposing light, to the action of an aqueous solution of a hydrazine substituted with a group selected from aromatic ring and carbamyl groups and developing a visible positive image in the element.

25 6. A photographic reversal process comprising forming a silver image in a gelatino-silver halide

emulsion layer, removing the silver image without affecting the remaining silver halide, subjecting the layer to the action of an aqueous solution of a hydrazine substituted with a group selected from aromatic ring and carbamyl groups as a nucleus-forming agent, and developing a positive image in the layer.

30 7. A photographic reversal process comprising forming a silver image in a gelatino-silver halide emulsion layer, removing the silver image without affecting the remaining silver halide, subjecting the layer to the action of an aqueous solution of semi carbazide as a nucleus-forming agent, and developing a positive image in the layer.

15 8. A photographic reversal process comprising forming a silver image in a gelatino-silver halide emulsion layer, removing the silver image without affecting the remaining silver halide, subjecting the layer to the action of an aqueous solution of a phenyl hydrazine as a nucleus-forming agent, and developing a positive image in the layer.

20 9. A photographic reversal process comprising forming a silver image in a gelatino-silver halide emulsion layer, removing the silver image without affecting the remaining silver halide, subjecting the layer to the action of an aqueous solution of hydrazino benzoic acid as a nucleus-forming agent, and developing a positive image in the layer.

25 10. A photographic reversal process comprising forming a silver image in a gelatino-silver halide emulsion layer, removing the silver image without affecting the remaining silver halide, subjecting the layer to the action of an aqueous solution of acetyl phenyl hydrazine as a nucleus-forming agent, and developing a positive image in the layer.

30 40 JOSEPH C. VILLE.

#### CERTIFICATE OF CORRECTION.

Patent No. 2,150,704.

March 14, 1939.

JOSEPH C. VILLE.

It is hereby certified that error appears in the printed specification of the above numbered patent requiring correction as follows: Page 2, second column, line 28, claim 9, strike out the syllable, words and syllable "tion of hydrazino benzoic acid as a nucleus-; and that the said Letters Patent should be read with this correction therein that the same may conform to the record of the case in the Patent Office.

Signed and sealed this 18th day of April, A. D. 1939.

Henry Van Arsdale

(Seal)

Acting Commissioner of Patents.